

# UNITED STATES PATENT OFFICE.

PIERRE E. HAYNES, OF BUFFALO, NEW YORK, ASSIGNOR TO THE LINDE AIR PRODUCTS COMPANY, A CORPORATION OF OHIO.

## EXPLOSIVE MIXTURE.

1,408,293.

Specification of Letters Patent. Patented Feb. 28, 1922.

No Drawing.

Application filed July 23, 1920. Serial No. 398,380.

To all whom it may concern:

Be it known that I, PIERRE E. HAYNES, a citizen of the United States, residing at Buffalo, in the county of Erie and State of New York, have invented certain new and useful Improvements in Explosive Mixtures, of which the following is a specification.

It has already been proposed to make an explosive by absorbing a highly volatile liquid oxidizing agent, such as these boiling at atmospheric pressure below the centigrade zero, for example, liquid oxygen or liquid ozone, in a highly absorbent combustible material, such as charcoal. Such a mixture is claimed in United States Patent No. 1,282,229.

These liquid oxidizing agents evaporate very rapidly at ordinary temperatures, and while the rate of evaporation is diminished by the presence of an absorbent, the oxidizing ingredient escapes at such a rate that if the charge is not fired within a short time, there will not be enough of the oxidizing component left to completely burn the combustible ingredient, in which event the efficiency of the explosive would be greatly impaired. For this reason, it is very important that a substantial excess of the oxidizing agent be absorbed in the combustible ingredient, and it is also important that the structure of the absorbent be such that the oxidizing agent will escape from it as slowly as possible.

In the prior patent referred to, the absorbent specifically claimed is balsa wood, preferably charred. While this material forms, when saturated with liquid oxygen or ozone, a mixture capable of exploding with practically maximum force for several minutes after its preparation, I have now found that the wood of certain other plants is much superior for this purpose. Examples of these plants are *Æschynomene aspera*, *Æschynomene cannabina*, *Æschynomene lagenaria* (Laureiro and Roxburgh), *Aralia* (Fatsia) and *Papyrifia* (Hook). Such plants are indigenous to the moist tor-

rid regions of India, China, Japan, and Formosa and are variously known as solah plant, sola, salah, solar, shota, spongewood, 50 hat plant, Tsuso, Tung-tsao, and pith plant. For the sake of brevity, all the above closely related plants will be hereinafter referred to as "sola."

While the sola wood may be merely dried 55 and then used as an absorbent, I prefer to carefully char it and to dry the char at a temperature of 110° C. shortly before using it. Obviously the char should be cooled before the low-boiling oxidizing liquid is absorbed in it. Evaporation of the liquid may be retarded by heat-insulating the charge, as by wrapping it in paper or the like, but satisfactory results may be obtained in most cases without the use of such heat-insulation. 65

My invention is not limited to the combination of the absorbent with the volatile oxidizing agent as other explosives, inert materials, or solid or liquid oxidizing or combustible ingredients may be added in 70 some cases, having due regard to the proper balance between oxidizing and reducing constituents, and the effect on this balance of the loss by evaporation of a portion of one or more of the constituents between the time 75 of preparing the charge and the time of firing it. The scope of the invention is only limited by the appended claims.

I claim:

1. An explosive mixture comprising dried sola wood and a liquid oxidizing agent.
2. An explosive mixture comprising carbonized sola wood and a liquid oxidizing agent.
3. An explosive mixture comprising dried sola wood and a liquid oxidizing agent boiling below the centigrade zero.
4. An explosive mixture comprising carbonized sola wood and a liquid oxidizing agent boiling below the centigrade zero. 90
5. An explosive mixture comprising carbonized sola wood and liquid ozone.

In testimony whereof I affix my signature.

PIERRE E. HAYNES.